

Patented Oct. 7, 1924.

1,510,855

# UNITED STATES PATENT OFFICE.

MARK W. MARSDEN, OF PHILADELPHIA, PENNSYLVANIA.

METHOD OF MAKING FIBROUS PULP FROM LOW-COST VEGETABLE MATTER.

No Drawing.

Application filed July 10, 1923. Serial No. 650,735.

To all whom it may concern:

Be it known that I, MARK W. MARSDEN, a citizen of the United States, residing at Philadelphia, in the county of Philadelphia and State of Pennsylvania, have invented certain new and useful Improvements in Methods of Making Fibrous Pulp from Low-Cost Vegetable Matter, of which the following is a specification.

10 The objects of my invention are to provide a method of producing fibrous pulp from waste or near waste vegetable growths such as corn stalks, cotton stalks, straw, etc., which may be used in making paper, explosives, artificial silk, and other products requiring pulp for their manufacture; to provide a method of producing such pulp by which the fibres will retain their natural strength and elasticity, and which the saccharine and other useful elements are separated from the fibres and recovered.

For convenience I will describe my invention as applied to the manufacture of pulp from corn stalks.

25 The first step is removal of dust and dirt and the second is removal of the pith. Both of these steps are old and may be effected by known means. The residue is subjected to a steam bath, at a temperature preferably not far above, or below 170° F., to reduce the material to a soft and moist state in which the fibres are easily separable, and is then passed through a shredding machine which may be of a known type. The shredded material is then passed to a fermentation vat where it should be kept at a temperature sufficient to produce fermentation but not sufficiently high to caramelize the saccharine contents. The fermentation may be hastened by use of any ordinary ferment such as yeast. The fermented mass is then distilled. The distillation carries over the sugars and carbo-hydrates and converts them into alcohol. The residue is placed in a closed digester and heated under pressure, an acid or alkali being added to aid in dissolving the encrusting matter. The heat and pressure should be only sufficient to effect the complete dissolution of the encrusting matter. The fibrous residue is then washed to eliminate all acid or alkali thereby leaving the pulp absolutely free from any foreign matter. The pulp is then ready for use and may be bleached, or colored as desired.

Obviously removal of the pith is not re-

quired in dealing with many of the fibrous vegetable materials.

I find that by use of the method, corn stalks, cotton stalks, straw and many other articles will produce a fibrous pulp in which the fibres retain their natural strength and elasticity and which, when used in paper making, produces paper of a quality far superior to that made from wood pulp and at far less cost. The pulp produced by my process is adapted for use for many purposes for which wood pulp is not adapted.

Having thus described my invention, what I claim as new and desire to secure by Letters Patent is:—

1. The herein described method of making fibrous pulp consisting in freeing the material from dust and other foreign matter; subjecting the material to a steam bath; shredding the softened material; fermenting the material, and distilling the fermented mass.

2. The herein described method of making fibrous pulp consisting in freeing the material from dust and other foreign matter; removing the pith; subjecting the material to a steam bath; shredding the softened material; fermenting the material, and distilling the fermented mass.

3. The herein described method of making fibrous pulp consisting in freeing the material from dust and other foreign matter; subjecting the material to a steam bath; shredding the softened material; fermenting the material; distilling the fermented mass; adding an acid or alkali to the fibrous residue; subjecting the product to heat, and washing the residue to remove the acid or alkali and other foreign matter.

4. The herein described method of making fibrous pulp consisting in freeing the material from dust and other foreign matter; subjecting the material to a steam bath; shredding the softened material; fermenting the material; distilling the fermented mass; adding an acid or alkali to the fibrous residue; subjecting the product to heat under pressure, and washing the residue to remove the acid or alkali.

In testimony whereof I have signed my name to this specification in the presence of two subscribing witnesses.

MARK W. MARSDEN.

Witnesses:

ELIZABETH GARRE,  
CHAS. E. POTTS.